

[54] **TOOL STEEL FOR HOT WORKING**

[75] Inventors: **Toshio Okuno, Yasugi; Rinzo Sasaki, Nagoya, both of Japan**

[73] Assignee: **Hitachi Metals, Ltd., Tokyo, Japan**

[22] Filed: **Nov. 27, 1974**

[21] Appl. No.: **527,740**

[30] **Foreign Application Priority Data**

Nov. 28, 1973 Japan..... 48-132737

[52] **U.S. Cl.**..... 75/128 B; 75/128 V; 75/128 W

[51] **Int. Cl.<sup>2</sup>**..... C22C 38/44; C22C 38/46; C22C 38/52

[58] **Field of Search** ..... 75/128 B, 128 W, 128 V

[56] **References Cited**

## UNITED STATES PATENTS

|           |         |                    |            |
|-----------|---------|--------------------|------------|
| 2,562,543 | 7/1951  | Gippert.....       | 75/128 V X |
| 2,644,747 | 7/1953  | Eder et al. ....   | 75/128 V   |
| 2,949,356 | 8/1960  | Hughs et al. ....  | 75/128 V X |
| 3,600,160 | 8/1971  | Simcoe et al. .... | 75/128 V X |
| 3,615,370 | 10/1971 | Ridal et al. ....  | 75/128 B   |

*Primary Examiner*—C. Lovell

*Assistant Examiner*—Arthur J. Steiner

*Attorney, Agent, or Firm*—Stewart and Kolasch, Ltd.

[57]

**ABSTRACT**

A tool steel for hot working containing, in weight percent, from 0.25 to 0.60% carbon, not more than 0.6% silicon, from 0.50 to 1.50% manganese, from 0.50 to 1.50% nickel, from 1.50 to 3.50% chromium, from 2.00 to 4.50% molybdenum, from 1.20 to 3.00 vanadium, from 0.50 to 5.00% cobalt, balance essentially iron and impurities, or containing, in weight percent, from 0.25 to 0.60% carbon, not more than 0.60% silicon, from 0.50 to 1.50% manganese, from 0.50 to 1.50% nickel, from 1.50 to 3.50% chromium, from 0.50 to 3.50% tungsten, from 1.50 to 3.00% molybdenum, from 1.20 to 3.00% vanadium, from 0.50 to 5.00% cobalt, balance essentially iron and impurities. This tool steel affords excellent high temperature mechanical strength, toughness, high temperature wear resistance, and heat check resistance.

**4 Claims, No Drawings**

## TOOL STEEL FOR HOT WORKING

## BACKGROUND OF THE INVENTION

## 1. Field of The Invention

This invention relates to a tool steel for hot working, which presents excellent high temperature mechanical strength, toughness, high temperature wear resistance and heat check resistance.

## 2. Description of The Prior Art

Hitherto, AISI H19 base steels of a high W-V-Co alloy system find a wide application as materials having the highest high temperature mechanical strength for meeting a demand arising from hot working which requires excellent mechanical strength and wear resistance at high temperature.

However, such steels suffer from disadvantages of often causing early stage or premature cracks due to the insufficient toughness in contrast to the excellent high temperature mechanical strength.

It is a principal object of the present invention to provide a tool steel for hot working, which present excellent toughness, high temperature wear resistance, heat check resistance and long service life superior to those of AISI H19 steel in addition to excellent high temperature mechanical strength similar to that of AISI H19 steel.

## SUMMARY OF THE INVENTION

According to the present invention, there are provided a tool steel for hot working containing, in weight

5 mium, from 0.50 to 3.50% tungsten, from 1.50 to 3.00% molybdenum, from 1.20 to 3.00% vanadium, from 0.50 to 5.00% cobalt, balance essentially iron and impurities. This tool steel affords excellent high temperature mechanical strength, toughness, high temperature wear resistance, and heat check resistance.

## DETAILED DESCRIPTION OF THE INVENTION

The tool steel according to the present invention has 10 a composition being added suitable amounts of carbide forming elements such as W, Mo and V to a low Cr—low Si-Mn-Ni-Co alloy system which is the fundamental components of this steel. In other words, the invention of this tool steel is: to improve resistance to the 15 temper softening as well as high-temperature strength due to precipitation hardening by adding a small amount of chrominum, a suitable amount of tungsten and molybdenum and a great amount of vanadium; to present a suitable degree of oxidative characteristic due to the addition of small amounts of chrominum and silicon, suitable amounts of molybdenum and manganese to thereby facilitate the formation of oxide films on the surface of a die due to the temperature rise in service; and to provide the aforesaid oxide film which is 20 intimate and adhesive, due to the addition of cobalt, nickel or tungsten, in an attempt to improve high-temperature wear resistance, corrosion resistance, rough-surface condition and heat check resistance due to the 25 resulting good lubricity and good heat insulating property; and to provide high resistance to the development or propagation of cracks by addition nickel to the composition of the steel.

Table 1

|                    | C    | Si   | Mn   | Ni   | Cr   | W    | Mo   | V    | Co   |
|--------------------|------|------|------|------|------|------|------|------|------|
| Present Invention  |      |      |      |      |      |      |      |      |      |
| Steel A            | 0.43 | 0.32 | 1.11 | 1.17 | 3.20 | —    | 2.88 | 2.32 | 3.65 |
| Steel B            | 0.40 | 0.24 | 0.78 | 0.85 | 2.86 | —    | 3.67 | 1.61 | 3.01 |
| Steel C            | 0.41 | 0.21 | 0.65 | 1.15 | 2.57 | 3.25 | 1.21 | 1.64 | 4.03 |
| Steel D            | 0.45 | 0.25 | 0.67 | 1.02 | 1.98 | —    | 2.46 | 1.55 | 2.13 |
| Prior Art          |      |      |      |      |      |      |      |      |      |
| Steel E (AISI H19) | 0.43 | 0.31 | 0.23 | —    | 4.35 | 4.38 | 0.42 | 2.02 | 4.32 |

percent, from 0.25 to 0.60% carbon, not more than 0.6% silicon, from 0.50 to 1.50% manganese, from 0.50 to 1.50% nickel, from 1.50 to 3.50% chromium, from 2.00 to 4.50% molybdenum, from 1.20 to 3.00% vanadium, from 0.50 to 5.00% cobalt, balance essentially iron and impurities; and a tool steel containing, in weight

50 Table 2 illustrates the heat treatment condition (target hardness of HRC45) and the high-temperature strengths, proving that the steels according to the present invention afford high-temperature strengths superior or equivalent to those of the conventional steels (AISI H19).

Table 2

|                   | Heat Treatment Condition |                     |       |          | High-temperature Strength (700°C)         |                                        |
|-------------------|--------------------------|---------------------|-------|----------|-------------------------------------------|----------------------------------------|
|                   |                          |                     |       |          | 0.2% yield strength (kg/mm <sup>2</sup> ) | tensile strength (kg/mm <sup>2</sup> ) |
| Present Invention | 1150°C                   | quenched, hardened, | 650°C | tempered | 38.2                                      | 53.9                                   |
| Steel A           | 1140°C                   | "                   | 650°C | "        | 36.9                                      | 52.1                                   |
| Steel B           | 1140°C                   | "                   | 650°C | "        | 37.4                                      | 52.7                                   |
| Steel C           | 1140°C                   | "                   | 650°C | "        | 35.9                                      | 51.2                                   |
| Steel D           | 1130°C                   | "                   | 650°C | "        | 37.8                                      | 53.0                                   |
| Prior Art         |                          |                     |       |          |                                           |                                        |
| Steel E           | 1140°C                   | "                   | 650°C | "        |                                           |                                        |

weight percent, from 0.25 to 0.60% carbon, not more than 0.60% silicon, from 0.50 to 1.50% manganese, from 0.50 to 1.50% nickel, from 1.50 to 3.50% chro-

mium, from 0.50 to 3.50% tungsten, from 1.50 to 3.00% molybdenum, from 1.20 to 3.00% vanadium, from 0.50 to 5.00% cobalt, balance essentially iron and impurities. This tool steel affords excellent high temperature mechanical strength, toughness, high temperature wear resistance, and heat check resistance.

Table 3

|                            | Critical Seizing Load (ratio) |
|----------------------------|-------------------------------|
| Present Invention, Steel A | 140                           |
| Present Invention, Steel B | 135                           |
| Present Invention, Steel C | 145                           |
| Present Invention, Steel D | 125                           |
| Prior Art, Steel E         | 100                           |

The heat treatment conditions remain the same for samples as given in Table 2. In those tests, samples of a column form were subjected to air oxidation treatment at 630°C beforehand, after which samples rotating were pressed on their end faces against a steel piece (counterpart) heated to 700°C, thereby determining the maximum load (critical load) which would not cause seizing, and then the critical loads were given as indexes in terms of the critical seizing load of a prior art steel being 100. As is apparent from this table, the steel according to the present invention presents a high critical seizing load. This is due to the protective and lubricating actions of an oxide film, intimate and adhesive, which has been formed on the surface of a sample of the steel according to the present invention, presenting one of the prominent features of the present invention.

Table 4 indicates the fracture toughness (ASTM E399 type sample) of the steels of the present invention.

Table 4

|                            | Fracture toughness kg/mm <sup>2</sup> /mm |
|----------------------------|-------------------------------------------|
| Present invention, Steel A | 251                                       |
| Present invention, Steel B | 262                                       |
| Present invention, Steel C | 259                                       |
| Present invention, Steel D | 267                                       |
| Prior art, Steel E         | 237                                       |

The heat treatment conditions used are the same as those given in Table 2. According to the present invention, nickel is added so as to promote the resistance against the development or propagation of cracks, presenting apparently higher fracture toughness than does the prior art steels, as well as a tendency not to cause cracks. This is also one of the prominent features of the present invention.

Table shows the results of tests given to samples of steels of the present invention for their heat check resistances, in which samples of dimensions of 15 mm × 25 mm were rapidly heated to 700°C and then quenched into water at 20°C. Then, such a cycle was repeated in 3,000 cycles.

As can be seen from this, the steels according to the present invention present excellent heat check resistance higher than or equivalent to those of the prior art steels.

Table 5

|                   | Number of cracks | Average depth of cracks(mm) | Maximum depth of cracks(mm) |
|-------------------|------------------|-----------------------------|-----------------------------|
| Present invention |                  |                             |                             |
| Steel A           | 112              | 0.14                        | 0.61                        |
| Present invention |                  |                             |                             |
| Steel C           | 114              | 0.14                        | 0.57                        |
| Prior art steel E | 120              | 0.18                        | 0.65                        |

The results shown above are attributable to the excellent high temperature strength, and high resistance against the development or propagation of cracks plus

protective and heat insulating properties of an oxide film formed on the surface of the steel according to the present invention.

Now, description will be given of the background of the composition of the steels according to the present invention.

The amount of carbon can vary between 0.25% and 0.60%, preferably, 0.30 and 0.50%. Carbon is necessary for maintaining desired hardenability, tempered hardness and high temperature hardness for steels according to the present invention. Carbon combines with carbide forming elements such as tungsten, vanadium and chromium to thereby form carbides, thus contributing to formation of fine crystals, desired wear resistance property, temper softening resistance and high temperature hardness of the steel. If the amount of carbon is excessive, then there results decrease in toughness, and thus the amount of carbon should be not more than 0.60%. On the other hand, if the amount of carbon is too small, then there results no intended effect of the addition of carbon, and thus the amount of carbon should be not less than 0.25%.

Silicon is present in amounts of not more than 0.60%. Silicon has a tendency to impair the characteristic to form heat-insulating-oxidized film formed due to the temperature rise in a die in service, and thus the amount of silicon should be minimized in this sense. However, considering the factors involved in a steel making process, the amount of silicon should be present in the above range.

The amount of manganese is between 0.50 and 1.50%. Manganese should be present for improving the characteristic to form a heat-insulating-oxidized film, that is, one of the prominent features of the present invention. If manganese is excessive in amounts, then there results lowered  $A_1$  transformation point and higher tempered hardness as well as lowered machinability. So, the upper limit of the amount of manganese is set to 1.50%. On the other hand, if the amount of manganese is too low, the intended effect of manganese can not be attained. Thus, the lower limit of the amount of manganese is 0.50%.

Nickel is present within the range of 0.50 to 1.50%. Nickel is necessary for affording excellent high temperature strength plus high toughness (which contribute to the resistance against the development of cracks) as well as for forming an adhesive, protective oxidized film due to the temperature rise in a die in service, thereby enhancing the heat check resistance and suppressing the formation of crack-developing nucleuses, with the aid of cobalt. If the amount of nickel is excessive, then there results lowered  $A_1$  transformation point, with the resulting increased tempered hardness which lowers machinability. Thus, the amount of nickel should be not more than 1.50%. On the other hand, if the amount of nickel is too low, then there results no desired effect of nickel added. Thus, the amount of nickel should be not less than 0.50%.

Chromium should be present within the range of from 1.50 to 3.50%, preferably, from 2.00 to 3.50%. Chromium is necessary for improving the high temperature strength and temper softening resistance as well as for affording a suitable characteristic of an oxidized film plus improved wear resistance due to the formation of carbides in combination with carbon. Chromium is further necessary for improving  $A_1$  transformation point effect and hardenability. In this sense, chromium is of supreme importance as an element for

the steels of the present invention. If the amount of chromium is too low, then there results insufficient oxidation resistance, with the resulting rough surface, lowered hardenability, lowered  $A_1$  transformation point and lowered wear resistance. Thus, the lower limit of the amount of chromium should be 1.50%. On the other hand, if the amount of chromium is excessive, then there results excessively high oxidation resistance, so that the steel fails to form a protective oxide film which is one of the major features of the present invention. In addition, chromium of an excessive amount promotes precipitation and cohesion of carbides, thus lowering the temper softening resistance and high temperature strength. Thus, the upper limits of chromium is set to 3.50%.

Tungsten is present within the range of from 0.50% to 3.50%, preferably, from 1.00 to 3.50%.

Tungsten is necessary because of its unique effect to improve the wear resistance due to the formation of carbides which hardly forms solid solutions upon heating for hardening as well as to increase the high temperature yield strength due to the precipitation of fine carbides in tempering, in addition to an attempt to provide an intimate oxidized film on the surface of a die due to a temperature rise in service. The effect of tungsten on the characteristics of an oxide film depends on the amounts of Cr, Mo, Si, Mn, Ni, Co. Thus, optimum combination of those elements can present excellent characteristics as shown in Table 3. Tungsten of an excessive amount tends to form large size carbides, thus causing lowered toughness. Thus, the amount of tungsten is limited to not more than 3.50%. On the other hand, tungsten of a too small amount, there results the failure to obtain the intended effect of tungsten. Thus, tungsten should be present in amounts of not less than 0.50%.

Molybdenum is present in the range of from 2.00 to 4.50%. Molybdenum is necessary for forming carbides to increase wear resistance and for improving the hardenability due to the formation of solid solution thereof into a matrix. In addition, molybdenum precipitates fine carbides at the time of tempering to increase the temper softening resistance as well as high temperature strength, in addition to its feasibility to form a protective oxidized film. If the amount of molybdenum is excessive, then there results lowered toughness. Thus, the upper limit of molybdenum is set to 4.50%. On the other hand, if molybdenum is too low in amounts, then there results no intended effect due to the addition of molybdenum. For accommodating the combined addition of tungsten, the upper limit of molybdenum is set to 3.00%, and the lower limit thereof is set to 0.50%. In this respect, in the case of the addition of molybdenum accompanying no tungsten, the range of the molybdenum level is between 2.50 to 350% while in the case of combined addition of molybdenum with tungsten, the amount of molybdenum should range from 1.00 to 3.00%.

Vanadium is present within the range of from 1.20 to 3.00%, preferably, from 1.20 to 2.50%.

Vanadium is necessary for forming a great amount of carbides which hardly form solid solutions to thereby improve the wear resistance and thermal stick resistance. In addition, vanadium forms solid solutions in a matrix at the time of heating for hardening, thus precipitating fine carbides which are hardly cohesive in tempering. This increases the softening resistance at elevated temperatures thus affording excellent high-tem-

perature yield strength, which is one of the outstanding features of the present invention. For this reason, vanadium should be present in a great amount for the steels of the present invention. In addition, the addition of 5 vanadium presents a fine grain size of crystals to improve toughness as well as to raise the  $A_1$  transformation temperature, thus improving high-temperature yield strength at elevated temperatures as well as heat check resistance. If the amount of vanadium is excessive, then there results large size carbides, thus lowering 10 toughness. Thus, the upper limit of vanadium is set to 3.00%. If the amount of vanadium is too low, then there results no intended effect due to the addition of vanadium. Thus, the lower limit of vanadium is set to 15 1.20%.

Cobalt is present within the range of from 0.50 to 5.00%, preferably, from 0.70 to 4.00%. Cobalt is necessary for affording excellent wear resistance at elevated temperatures. This is because of the formation of a 20 protective oxide film which is intimate and adhesive, at the time of the temperature rise in a die in service. This prevents its metallic contact with work pieces, preventing the temperature rise in a die as well as presenting high wear resistance. In addition, cobalt presents a heat 25 insulating property due to the formation of an oxide film, improvement in heat check resistance due to the protective action of the film, and suppression of formation of crack developing nucleuses. The aforesaid effect of cobalt differs by the added amount of nickel, 30 tungsten, molybdenum and the like. Thus, in the case of the present invention, cobalt should not be added in a great amount. If the amount of cobalt is excessive, then there results lowered toughness. Thus, cobalt should be present in amounts of no more than 5.00%. 35 On the other hand, if the amount of cobalt is too low, then there may not attain the intended effect due to the addition of cobalt. Thus, cobalt should be present in amounts of no less than 0.50%.

As is apparent from the foregoing description, the 40 steels for hot working according to the present invention present high resistance against the development or propagation of cracks, excellent high wear resistance and seizing resistance due to the formation of a dense and adhesive oxide film by temperature rise at hot 45 working. In addition, the steels of the present invention suppress the formation of the initial cracks or crack developing nucleuses as well as insure a long service life with consistent high performances.

What is claimed is:

50 1. A tool steel for hot working consisting essentially of, in weight percent, from 0.25 to 0.60% carbon, not more than 0.6% silicon, from 0.50 to 1.50% manganese, from 0.50 to 1.50% nickel, from 1.50 to 3.50% chromium, from 2.00 to 4.50% molybdenum, from 1.20 to 3.00% vanadium, from 0.50 to 5.00% cobalt, balance essentially iron and impurities.

2. A tool steel for hot working consisting essentially of, in weight percent, from 0.03 to 0.50% carbon, no more than 0.60% silicon, from 0.50 to 1.00% manganese from 0.70 to 1.40% nickel, from 2.00 to 3.50% chromium, from 2.5 to 3.50% molybdenum, from 1.20 to 2.50% vanadium, from 0.70 to 4.00% cobalt, balance essentially iron and impurities.

60 3. A tool steel for hot working consisting essentially of, in weight percent, from 0.25 to 0.60% carbon, not more than 0.60% silicon, from 0.50 to 1.50% manganese, from 0.50 to 1.50% nickel, from 1.50 to 3.50% chromium, from 0.50 to 3.50% tungsten, from 1.50 to

3.00% molybdenum, from 1.20 to 3.00% vanadium, from 0.50 to 5.00% cobalt, balance essentially iron and impurities.

4. A tool steel for hot working consisting essentially of, in weight percent, from 0.30 to 0.50% carbon, no more than 0.60% silicon, from 0.50 to 1.00% manga-

nese, from 0.70 to 1.40% nickel, from 2.00 to 3.50% chromium, from 1.00 to 3.50% tungsten, from 1.00 to 3.00% molybdenum, from 1.20 to 2.50% vanadium, from 0.70 to 4.00% cobalt, balance essentially iron and impurities.

\* \* \* \* \*

10

15

20

25

30

35

40

45

50

55

60

65